

March 12, 1935.

H. J. BILLINGS

1,994,093

SOUND RECORD

Filed July 17, 1929



Inventor  
Howard J. Billings  
by Roberts, Cushman & Woodbury  
Attnys.

## UNITED STATES PATENT OFFICE

1,994,093

## SOUND RECORD

Howard J. Billings, South Acton, Mass., assignor  
to Arthur D. Little, Incorporated, Cambridge,  
Mass., a corporation of Massachusetts

Application July 17, 1929, Serial No. 378,893

11 Claims. (Cl. 18—48.3)

This invention relates to improvements in sound records and its chief object is to provide a sound record having a backing or core upon which is provided at one or both sides a record sheet consisting of a base of moldable compound in sheet form and a coating which forms the playing surface. In the preferred form of record the grooves are impressed into the base and are completely lined with the coating. A further object

10 is to provide a method of making such a record.

A further object of this invention is to provide, in a sound record, a recording sheet consisting of a base of molding compound in sheet form, comprising a thermoplastic binder and felted fibrous material intimately associated throughout the body of the compound, and a coating for said base comprising a thermoplastic binder, a filler and an abrasive in approximately equal parts.

Another object of this invention is to provide, 20 in a sound record, a core or backing consisting of a plurality of laminated sheets certain of said sheets being of moldable compound comprising a thermoplastic binder and a filler intimately associated throughout the body of the compound, 25 and other of said sheets having less or no binder therein.

Other objects of this invention will appear from an examination of the following specification taken in connection with the accompanying drawing which forms a part thereof and in which

30 Fig. 1 is a diagrammatic view in section of a sound record embodying one form of this invention prior to the formation of record groove therein, the several layers being shown separated for clearness;

35 Fig. 2 is an enlarged sectional view of a portion of a record blank before the record grooves are formed therein;

40 Fig. 3 is an enlarged sectional view of a portion of the sound record shown in Figs. 1 and 2 after the record grooves have been formed therein;

45 Fig. 4 is a sectional view similar to that shown in Fig. 2 of said record sheet alone; and

Fig. 5 is a sectional view of a sound record 50 embodying another form of this invention.

Sound records produced in accordance with the methods now or formerly in use are generally frangible and unbendable so that they crack or break fairly readily when subjected to the general 55 course of handling or when shipped through the mail. On the other hand records made according to this invention may be handled or shipped without the necessity of expensive packing, may be dropped upon the floor without injury to the playing surfaces and after being so treated regain their original condition without developing any surface cracks or hair lines in the playing surfaces which would have a deleterious effect upon their use as sound records.

60 I am well aware of the fact that there are now

two ways of manufacturing sound records of a flexible type which methods are briefly first, to coat or paint sheets of cardboard or paper with shellac, synthetic resin or other shellac-like material, and form the record grooves in the coating, and second, to incorporate shellac in paper by repeated coatings or dippings and use the paper so treated as a record sheet.

Neither of these methods, however, produces satisfactory records. The coating is always liable to develop cracks or hair lines on bending or dropping if it be built up to a thickness sufficient to receive and retain satisfactory playing surface impressions, a condition which cannot be avoided by providing a very thin coating of the resinous surface because such a coating would not receive and retain a satisfactory playing surface and would not have the requisite surface strength to prevent the record from cracking if bent or dropped.

Sound records, particularly those of the disk type now almost universally used, made in accordance with this invention have a smooth playing surface and the walls of the sound grooves are so strong that they will not under ordinary use break down and permit the needle to jump across from one groove to another, possess toughness, flexibility without producing hair lines or cracks in the playing surface, can be made economically and when finished have a high glaze upon the outer surfaces. Moreover the record is much lighter than the sound records commercially manufactured at the present time. Thus a ten-inch record of my invention weighs between three and four ounces while the average commercial record of the same diameter weighs not less than seven ounces.

As shown in the drawing the sound record 10 comprises a backing or core 11, (Fig. 1) and a record sheet 12. The backing 11 in the first embodiment is a laminated structure comprising a plurality of combining sheets 15, preferably of a moldable compound, and filling sheets 16, preferably of paper. These sheets are preferably, though not necessarily, arranged alternately as shown in Fig. 1. The record sheet 12 comprises a base 20 consisting of an uncoated sheet of moldable compound and a thin coating 21 upon the outer surface thereof. The record grooves 25 in the recording surface of the coating 21 are also impressed into the base 20, the coating 21 completely lining the grooves, whereby the walls or ridges 26 separating the grooves 25 are completely covered by the coating 21 and interiorly reinforced near the bottoms by the base 20, as is clearly shown in Fig. 3.

The combining sheets 15 and bases 20 (before coating) are preferably made by a process of pulping fibrous material in association with a thermoplastic binder. The details of this process per se

5

10

15

20

25

30

35

40

45

50

55

60

form no part of the present invention and the process will here be described briefly as follows.

The thermoplastic binder, preferably shellac alone or in combination with other thermoplastic material is kneaded under heat with wet fibrous material until a substantially uniform mass is obtained, the resultant mass is broken down to a pulp by the addition of water followed by a final fibration in a paper mill beater and the pulp is then felted into continuous sheets on paper mill equipment.

As a result of this process the binder and fibrous material are intimately associated throughout the mass, the binder being uniformly dispersed in the form of discrete particles in an amount in excess of that which can be absorbed by the fibrous material.

The base 20 of the record sheet may be prepared according to the foregoing method using the following proportion of materials.

*Formula #1*

|                                     | Per cent |
|-------------------------------------|----------|
| Shellac                             | 48       |
| Graphite                            | 25       |
| Carbon black                        | 2.5      |
| Rosin                               | 2.5      |
| Paper pulp {kraft 25%}<br>news 75%} | 22       |

30 It will be understood that the above formula can be modified in several respects both as to the materials and the proportions used. Thus in place of shellac and rosin, shellac alone may be used or other resins or thermoplastic material 35 may be used, either alone or in combination, suitable for a playing surface, the graphite and carbon black may be replaced by other fillers and pigments and other fibrous materials may be used.

40 The combining sheets 15 may be made by the same formula, or, if greater economy in materials is desired, the following composition has been found suitable:

*Formula #2*

|                                                     | Per cent |
|-----------------------------------------------------|----------|
| Thermoplastic binder {shellac 25%}<br>rosin 75%}    | 66       |
| Fibrous material {kraft pulp 60%}<br>news pulp 40%} | 34       |

50 This composition is here given merely as an example of the many that might be used, and obviously the invention is not limited thereto.

55 The coating 21 may be prepared with varying formulae and in many ways, but I have found the following to give very satisfactory results. The ingredients and proportions are as follows: (the proportions being by weight).

*Formula #3*

|                                                                                                  | Per cent |
|--------------------------------------------------------------------------------------------------|----------|
| Binder; shellac or other thermoplastic material that will produce a satisfactory playing surface | 30       |
| Abrasive filler; rotten stone or similar material                                                | 34       |
| Filler to give body; china clay or the like                                                      | 34       |
| Pigment; such as carbon black                                                                    | 2        |

70 The ingredients are mixed together on rolls and sheeted in the well known and customary manner.

75 The record sheet 12 is made by applying to the base 20 the coating 21 which step may be performed in either of the following methods which may be differentiated roughly as dry and wet. In the first of these methods the coating composition

is ground dry to a powder which is dusted upon the base sheet 20 and caused to adhere by passing the sheet through an oven so that the powder is incipiently fused. In the other method, the coating composition is ground in water, and to it is added, if necessary, more shellac to enhance its molding properties. The result is a paint having adhesive, binding and molding properties particularly suitable for coating the base sheet 20. The paint may be applied as a liquid to the base by means of a brush or in any desired manner, and sets upon drying.

The backing or core 11, when made of laminae, as shown in Fig. 1, consists of alternately arranged disks of combining and filling sheets. The filling sheets are preferably formed of fairly dense or hard paper, e. g. kraft paper, to avoid the tendency of the finished core to spring back after the final pressure used for making the core is relieved. The filling sheets may be of paper impervious to moisture, such as paper having a waterproofing filler of asphalt or similar material. One satisfactory arrangement is to provide five filling disks and four combining disks. These may be assembled as disks when the sound record is to be made or may be assembled and formed, previous to the making of the record, into a unit, by the use of heat and pressure either as disks or as sheets, the backing being cut as a unit disk from the sheet if the second procedure is followed.

From the record sheet are cut disks which, when manufacturing a sound record having two playing surfaces, are placed upon each side of the backing, whether preformed or not, with the coated surfaces exposed. The assembled article is then placed between two dies each supporting a stamper which constitutes a matrix of the record grooves which are to be impressed into the sheet. The dies are steam heated and compress the article with a pressure of from 2000 to 4000 pounds per square inch, being so held for a period of predetermined length. The dies are then chilled by cold water and after the completed record has been sufficiently cooled the pressure is released and the record removed.

The grooves 25 thus formed in the recording surfaces are impressed into the base 20 and completely lined by the coating 21 so that the walls 26 of the grooves are very strongly reinforced at their roots as shown in Fig. 3. In this feature resides one of the differences between my record and those previously made wherein the coating upon the paper base was necessarily made of sufficient thickness to receive the grooves and the grooves were formed wholly in the coating and their walls were formed by the coating alone. It has therefore been previously thought that since the walls of the grooves must be formed by the coating alone, the coating should contain flock or other fibrous material which would give the necessary strength to the walls to prevent the needle from breaking through after the record has been in use. While this procedure did tend to strengthen the walls, it was objectionable in that it was found practically impossible to prevent the flock or other fibrous material from being exposed or so thinly covered in spots that it was picked up by the needle when the record was used.

70 The grooves 25 are about 1/300th of an inch in depth in accordance with the usual practice, and since the coating 21 is usually less or not substantially greater than the depth of the grooves it is obvious that satisfactory grooves could not be

formed in the coatings alone. The walls 26 of the grooves are in places very thin as when the sinuosities of the adjacent grooves are such that a particular portion of one groove is brought into very close relation to a particular portion of the adjacent groove. The needle bears against the roots of the groove walls and hence the reinforcement of the coating which forms the wall by the fibrous stratum of the base as shown in Fig. 3, strengthens the wall and prevents the needle from breaking it down. The strength of the walls so made is such that it is possible to increase the number of grooves per inch and thus provide a record having a greater playing surface without increasing the diameter of the record disk.

The thermoplastic binder extends through the entire mass of the record sheets and backing and when cooled securely unites them. Nevertheless, due to the variance in the amount of thermoplastic binder in the various strata of the sheets 20 the record is flexible and may be bent without danger of cracking or developing hair lines in the playing surface.

The heat and pressure in the die acts upon the thermoplastic binder in the base of the record sheet and in combining sheets, as well as forming the record grooves in the coating. The binder while intimately associated with the fibers throughout the mass of each sheet is present in an amount greatly in excess of that which can be absorbed by the fibers and flows outwardly from the fibers to the surfaces. Thus each record sheet 12 now comprises (see Fig. 3) a base or substratum *a* of thermoplastic material having 30 felted fibers uniformly distributed throughout its mass, a subsurface stratum *b* of fiber-free thermoplastic material intimately united to one side of the first stratum and wholly encasing the fibers thereof, and a superstratum *c* comprising a superficial coating of thermoplastic material containing fillers and integrally united to the subsurface stratum. The thermoplastic material flowing from the fibers of the base toward the backing serves to bond the backing to the record sheet. In the same way the thermoplastic material flowing outwardly from the fibers of the combining sheets serves to bond the laminae of the backing together.

The thermoplastic material forming the fibre-free stratum *b* is, as pointed out above, suitable for a playing surface and being fused to the coating prevents the entry of fibres into the surfaces of the grooves, and in case the coating should wear in the groove will form a playing surface. Moreover, this stratum prevents the escape of any of the binder in the coating 21 into the base.

When it is desired to make a sound record having only one playing surface, a suitable sheet is substituted for a record sheet on one side of the backing. In other respects the procedure described above and the product obtained thereby are the same.

In place of the laminated core, there might be employed a solid non-resilient core 30, (Fig. 5) 65 which, when assembled with the record sheet 12<sup>a</sup>, would give a very satisfactory record so far as playing is concerned but which would not have the bending and flexible qualities of a record made in accordance with the above invention.

It will be understood that, while the word "shellac" is used throughout the specification and claims, I intend to include thereby all gums, natural resins and phenolic condensation products which are shellac-like in function.

75 One of the procedures for making a record ac-

cording to my invention, which I have found to produce a satisfactory record, is the following and is here set forth as illustrative not as limitative.

The record is composed of two surface or record sheets and a core of nine laminae made up of five sheets of filling paper of ten point thickness, separated by four combining sheets of ten point thickness and made according to Formula No. 2. The record sheets comprise bases made according to Formula No. 1 to which is applied coating made 10 according to Formula No. 3 by either of the before described methods. I have found a very thin, flexible, non-cracking coating of five grams to a ten-inch disk of moldable compound to give a satisfactory result. For the filling paper a hard 15 finished kraft paper of ten point thickness is used. Each of the various sheets is substantially as dry as is feasible under working conditions.

The first step in stamping the record from this material is to cut from these sheets disks of the 20 desired diameter, properly centered by a hole punched in the middle and then assemble them as in Fig. 1. The record blank so formed is placed between stampers mounted on the dies of a press, preferably a hydraulic press. The record blank 25 is subjected to a pressure of from 2000 to 4000 pounds per square inch, during which time the blank is heated by steam circulated through the dies under a pressure of from 80 to 100 pounds. The temperature of the stampers is about 300° F. 30 less whatever loss of heat may occur through radiation. The time of heating and of bringing the press to maximum pressure should be from 15 to 20 seconds. The steam is turned on when the press is started, and as soon as the maximum pressure has been applied the steam is turned off and cold water run through the dies to cool the stamps. The time of cooling usually requires about 20 seconds. As soon as the dies have been cooled, as above described, the pressure may be 35 released and the record removed. All that remains to be done to finish this record is the trimming and finishing of the edges.

Unless the foregoing procedure is closely adhered to, difficulty may be experienced in having 45 the records stick to the stampers, due in part to the tendency of the shellac to undergo decomposition if heated for a time appreciably longer than with the foregoing temperatures.

Moreover due to the large amount of thermoplastic material throughout the record there will be a tendency for the record to contract as it cools. This tendency is exerted in all three dimensions, length, breadth, and thickness, and since the record is held firmly in the dies a strain 55 or tension is set up. This strain or tension is of course released when the press is open and the record springs free from the matrices. The presence of water or moisture in the press will cause the records to stick, and unless the moisture is removed as soon as discovered the records will be spoiled.

I claim:

1. A record sheet adapted to receive and retain record-grooves, said sheet being made of an 65 uncoated sheet of felted fibers containing in its interior and within the confines of its surface enough shellac to flow outwardly upon fusion under heat and pressure so as to form a continuous outer surface wholly encasing the fibers, and a 70 superficial coating containing shellac and filler on said sheet.

2. A record sheet adapted to receive and retain record-grooves, said sheet being made of an uncoated sheet of felted fibers containing in its in- 75

terior and within the confines of its surface enough shellac-like material adapted to produce a playing surface to flow outwardly upon fusion under heat and pressure so as to form a continuous outer surface wholly encasing the fibers, and a superficial coating containing shellac and filler on said sheet.

3. A record sheet adapted to receive and retain record-grooves, said sheet being made of an uncoated sheet of felted fibers containing in its interior and within the confines of its surface enough thermoplastic binder to flow outwardly upon fusion under heat and pressure so as to form a continuous outer surface wholly encasing the fibers, and a superficial coating containing shellac and filler on said sheet.

4. A record sheet adapted to receive and retain record-grooves, said sheet comprising an uncoated base of molding compound in sheet form including a thermoplastic binder and felted fibrous material intimately associated with the binder throughout the mass of the compound, the amount of binder being approximately double the amount of fibrous material and a superficial coating containing thermoplastic binder and an abrasive upon the base.

5. The method of making a sound record from a record sheet containing a base of felted fibers and thermoplastic material, the latter in an amount in excess of that which can be absorbed by the fibers, and a superficial coating of thermoplastic material suitable for a playing surface, which comprises assembling said record sheet and a backing sheet, and subjecting the assembled sheets to heat and pressure to cause thermoplastic material to flow outwardly from the felted fiber of the base and form a fiber-free subsurface layer between the fibers and the coating and a bond between said base and backing sheet.

6. The method of making a sound record from a backing and a record sheet comprising a base of felted fibers and thermoplastic material, the latter in an amount in excess of that which can be absorbed by the fibers, and a superficial coating of thermoplastic material suitable for a playing surface, which includes as steps applying said record sheet to the backing with the coated side outward and subjecting the backing and record sheet to heat and pressure to cause thermoplastic material to flow outwardly from the felted fibers of the base, thereby forming a fiber-free subsurface layer between the fibers and the coating, and simultaneously bonding the base to the backing.

7. The method of making a sound record from a backing consisting of laminæ of combining sheets of felted fibers and thermoplastic material, the latter in an amount in excess of that which can be absorbed by the fibers, and filling sheets, and a record sheet comprising a base of felted fibers and

thermoplastic material suitable for a playing surface, the latter in an amount in excess of that which can be absorbed by the fibers, and a superficial coating of thermoplastic material suitable for a playing surface, which includes as steps assembling said laminae of the backing and said record sheet and subjecting the same to heat and pressure to cause thermoplastic material to flow outwardly in both directions from the felted fiber in each combining sheet in the base of the record sheet, thereby bonding all the sheets together and simultaneously forming a fiber-free subsurface layer of said thermoplastic material between the fibers of the base and the coating.

8. A record sheet adapted to receive and retain record grooves, said record sheet comprising a substratum of uncoated felted fibers containing in its interior and within its confines enough thermoplastic binder to flow outwardly upon fusion under heat and pressure so as to form a continuous subsurface stratum wholly encasing the fibers of the substratum, and a surface stratum of thermoplastic material containing a filler.

9. A sound record blank having at one side a record sheet comprising a substratum of uncoated felted fibers containing in its interior and within its confines enough thermoplastic binder to flow outwardly upon fusion under heat and pressure so as to form a continuous subsurface stratum wholly encasing said substratum, said substratum being capable of providing record grooves having walls which are internally reinforced by its fibrous structure, and a superficial coating of material on the outer surface of said record sheet suitable for a playing surface.

10. A sound record blank comprising a laminated backing built up of combining sheets and filling sheets interposed between said combining sheets, said combining sheets comprising uncoated felted fibrous material containing in its interior and within its confines enough thermoplastic binder to flow outwardly upon fusion under heat and pressure so as to form a continuous stratum wholly encasing the fibers of the combining sheets and operative to bond the filling and combining sheets together to provide a laminated structure.

11. A sound record blank comprising a record sheet adapted to receive and retain record grooves, said record sheet comprising a substratum of uncoated felted fibers containing in its interior and within its confines enough thermoplastic binder to flow outwardly upon fusion under heat and pressure so as to form a continuous subsurface stratum wholly encasing the fibers of the substratum, and a laminated backing adjoining said record sheet, said backing comprising a plurality of combining sheets and filling sheets interposed between said combining sheets.

HOWARD J. BILLINGS.

60